

1

2,853,395

## CELLULOSIC SPONGE PROCESS

Robert Otto Osborn, Snyder, N. Y., assignor to E. I. du Pont de Nemours and Company, Wilmington, Del., a corporation of Delaware

No Drawing. Application March 12, 1954  
Serial No. 415,971

2 Claims. (Cl. 106—122)

This invention relates to the production of artificial sponge. More particularly, it relates to the production of cellulosic sponge from cellulosic solutions or dispersions such as viscose.

In the usual manufacture of artificial cellulosic sponge, a pasty mass is prepared by mixing together viscose (cellulose xanthate dissolved in caustic soda solution), strength-giving fibers such as hemp or jute, and a soluble pore-forming substance such as sodium sulfate decahydrate. This mixture is placed in molds and coagulated and regenerated by means of heat and/or the chemical action of a suitable solution. After coagulation and regeneration have been completed, the pore-forming substance is melted or washed from the mass; and the resulting cellulosic sponge-like material is washed, dried and/or subjected to other finishing treatments, and then cut into appropriate blocks. A well formed sponge produced in accordance with the process just described will have fibers uniformly distributed throughout the sponge structure. However, even though the fibers are incorporated in the viscose with thorough mixing, the fibers have a marked tendency to aggregate in clumps or "knots" which result in undesirable stiff lumps in an otherwise soft sponge.

An object of this invention, therefore, is to provide a process for producing substantially knot-free cellulosic sponges. Another object is to provide steps for the uniform and stable distribution of reinforcing (strength-giving) fibers in a cellulosic sponge derived from viscose. The foregoing and other objects will more clearly appear hereinafter.

These objects are realized by the present invention which, briefly stated, comprises dispersing reinforcing fibers in a liquid medium selected from the group consisting of water and dilute aqueous caustic soda solution, and thereafter mixing the resulting dispersion with cellulose xanthate whereby to form viscose having reinforcing fibers uniformly distributed therethrough. The fiber-containing viscose so produced is thereafter treated by known methods to form a cellulosic sponge structure; e. g., a soluble pore-forming substance is incorporated in the fiber-containing viscose to form a sponge mix which is placed in molds and is then coagulated and regenerated, after which the pore-forming substance is removed and the resulting cellulosic sponge structure is washed and dried.

Reference is made to United States Patent No. 2,295,823 for a full disclosure of the materials as well as the amounts and conditions that may be used in connection with the steps of the process of this invention for producing cellulosic sponges from viscose. It is to be understood, of course, that any fiber that will impart strength to the sponge structure, and that any suitable pore-forming substance, may be employed herein in place of the specific fibers and soluble pore-forming substances disclosed in United States Patent No. 2,295,823. Moreover, coagulation and/or regeneration of the sponge mixture may be effected by any known expedient, and the

2

resulting sponge structure may be subjected to any desired finishing treatments.

The following example of a preferred embodiment further illustrates the principles and practice of this invention. Parts and percentages are by weight unless otherwise indicated.

### EXAMPLE

Ingredients are added to a mixer in the following order and mixed as specified:

- (1) 550 parts of water.
- (2) 93 parts of hemp fiber (cut into the desired length), added over a period of 2-3 minutes, with the mixer operating.

(3) 50 parts of 26% caustic soda solution.

(4) Mix for approximately 10 minutes.

(5) 1214 parts of cellulose xanthate added.

(6) Mix for approximately 30 minutes.

(7) Add 1250 parts of water with continuous mixing over a period of 2 hours.

(8) Add 16,600 parts of crystals of sodium sulfate decahydrate of the appropriate size or range of sizes to give the desired pore structure and mix together thoroughly.

The completed sponge mix is then placed in molds and is coagulated and regenerated by means of heat, as described in United States Patent No. 1,909,629 (Pfannenstiel et al.) or No. 2,133,810 (Craigue). The coagulated sponges are removed from the molds, washed, bleached, purified, dried and/or subjected to other finishing treatments, and then cut into suitable blocks.

Examination of the sponge blocks reveals that knots are practically eliminated by the method of this invention. Knot values for sponges made according to the old method (adding fibers to the viscose) are given for comparative purposes. See Table I.

Table I

KNOTS IN SPONGES

| Size of Sponge Block                                 | Number of Sponge Blocks Examined | Total Number of Knots Found |                      |
|------------------------------------------------------|----------------------------------|-----------------------------|----------------------|
|                                                      |                                  | Old Method                  | New Method           |
| 1" x 3" x 4½"                                        | 95                               | 5.....                      |                      |
| 1" x 3" x 4½"                                        | 193                              |                             | 0.                   |
| 1½" x 3½" x 5½"                                      | 1,680                            | 58.....                     |                      |
| 1½" x 3½" x 5½"                                      | 1,683                            |                             | 0.                   |
| Oval-shaped sponge cut in half:                      |                                  |                             |                      |
| 2" x 4½" x 7"                                        | 28                               | 1.....                      |                      |
| 2" x 4½" x 7"                                        | 28                               |                             | 0.                   |
| 2 large blocks cut into strips $\frac{3}{8}$ " wide. |                                  | 58 or 26.5 per block.       |                      |
| 6 large blocks cut into strips $\frac{1}{2}$ " wide. |                                  |                             | 15 or 2.5 per block. |

By reason of the improvement of the present invention, the reinforcing fibers are thoroughly wetted and dispersed before the mix becomes thick and viscous due to the addition of the cellulose xanthate. Another advantage of the present invention is that fibers difficult to fluff and, hence, heretofore rejected as reinforcing fibers in sponge structures, can now be used.

I claim:

1. In the manufacture of cellulosic sponges wherein viscose, reinforcing fibers, and a pore-forming substance are combined to form a sponge mix which is then coagulated, regenerated, and purified to form a sponge structure, the improvement which comprises the steps of dispersing said reinforcing fibers in a liquid medium consisting of a member selected from the group consisting of water and dilute aqueous caustic soda solution, and thereafter mixing the resulting dispersion with cellulose

xanthate, whereby to form viscose having reinforcing fibers uniformly distributed therethrough.

2. The process according to claim 1 wherein said liquid medium is dilute aqueous caustic soda solution.

|           |                        |               |
|-----------|------------------------|---------------|
| 2,266,313 | Ehlers et al. -----    | Dec. 16, 1941 |
| 2,331,936 | Schlosser et al. ----- | Oct. 19, 1943 |
| 2,354,260 | Haney et al. -----     | July 25, 1944 |
| 2,495,237 | Petiton -----          | Jan. 24, 1950 |

**References Cited in the file of this patent**

**UNITED STATES PATENTS**

|           |              |                |
|-----------|--------------|----------------|
| 1,974,393 | Mostny ----- | Sept. 18, 1934 |
|-----------|--------------|----------------|

|         |       |
|---------|-------|
| 438,851 | ----- |
| 866,132 | ----- |

**FOREIGN PATENTS**

|                     |               |
|---------------------|---------------|
| Great Britain ----- | Nov. 25, 1935 |
| France -----        | June 18, 1941 |